

## 1

3,136,631

**VANADIUM-COLUMBIUM ALLOYS**  
 Stanley T. Wlodek, Niagara Falls, N.Y., assignor to  
 Union Carbide Corporation, a corporation of New  
 York  
 No Drawing. Filed Apr. 27, 1960, Ser. No. 24,887  
 4 Claims. (Cl. 75—134)

The present invention relates to vanadium-columbium alloys possessing exceptional high temperature strength and resistance to a variety of corrosive media and in addition possess resistance to atmospheric oxidation sufficient to enable them to be fabricated at elevated temperatures by conventional techniques without the necessity of elaborate atmospheric controls.

It is an object of this invention to provide an alloy having excellent tensile, and stress-rupture strength at elevated temperature.

It is another object of this invention to provide an alloy having high resistance to corrosive media such as wet chlorine gas; and boiling sulfuric, nitric and hydrochloric acid.

It is a further object of this invention to provide an alloy having a superior strength-to-weight ratio.

It is still another object of this invention to provide an alloy of exceptional mechanical strength having in addition outstanding resistance to aqueous corrosive media and sufficient resistance to atmospheric corrosion, particularly air oxidation, with the result that high temperature fabrication can be performed thereon in air by conventional means.

These and other objects and advantages will become apparent from the following description.

The invention broadly consists of a new and improved high strength, corrosion resistant alloy containing from about 15 to 60 weight percent columbium up to 25 weight percent titanium; 0 to 30 weight percent of at least one element of the group consisting of molybdenum, tantalum, tungsten and iron; 0 to 10 weight percent of at least one element of the group consisting of chromium, aluminum, cobalt, nickel, zirconium and hafnium; 0 to 5 weight percent of at least one element of the group consisting of silicon, beryllium, and the lanthanides; less than 1 weight percent in the aggregate carbon, oxygen, and nitrogen; and the balance consisting essentially of vanadium, the vanadium comprising at least about 30 weight percent of the alloy and the sum of vanadium and columbium to comprise at least about 50 weight percent of the alloy.

## 2

The preferred alloy consists of 25 to 40 weight percent columbium; 5 to 15 weight percent titanium; 15 to 25 weight percent of at least one element of the group consisting of molybdenum, tantalum and tungsten when present; 0 to 5 weight percent of at least one element of the group consisting of chromium, aluminum, cobalt, nickel, zirconium and hafnium; 0 to 3 weight percent of at least one element of the group consisting of silicon, beryllium and the lanthanides, less than 1 weight percent in the aggregate of carbon, oxygen and nitrogen; and the balance consisting essentially of vanadium, the vanadium comprising at least about 40 weight percent of the alloy and the sum of vanadium and columbium to comprise at least about 65 weight percent of the alloy.

The elements which are added to the binary columbium-vanadium system are classified in the following groups which are characterized by their degree of solubility in the columbium-vanadium binary alloy and the following general characteristics commonly associated with their presence in this binary system.

## HIGHLY SOLUBLE ELEMENTS

Titanium additions increase oxidation resistance, improve corrosion resistance in aqueous oxidizing media and up to 7 weight percent titanium improves the mechanical properties of the alloy. Titanium also tends to stabilize vanadates.

Molybdenum, tantalum and tungsten additions are employed to impart corrosion resistance and to provide better mechanical properties.

## INTERMEDIATELY SOLUBLE ELEMENTS

The addition of chromium, aluminum, cobalt, nickel, zirconium, iron and hafnium will increase oxidation resistance of the binary columbium-vanadium system and since these elements differ in atomic size and lattice, they also tend to increase the tensile strength of the alloy. These elements also tend to reduce the amount of  $V_2O_5$  formed under oxidizing conditions.

## LOW SOLUBILITY ELEMENTS

Silicon, beryllium and the elements of the lanthanide series are strong oxide formers.

When one or more elements characterized by high solubility in the vanadium-columbium matrix, in particular, titanium, molybdenum, tantalum and tungsten are added, an increase in the resistance of the resulting alloy to pure

Table I

## RESULTS OF CORROSION TESTS ON VANADIUM ALLOYS

[As-cast buttons]

| Composition, percent by weight                          |    |     | Rm.<br>temp.,<br>wet Cl <sub>2</sub> | Boiling<br>65%<br>NH <sub>4</sub> Os | Corrosion rate, mils./year |     |        |                                        |    |     |     |
|---------------------------------------------------------|----|-----|--------------------------------------|--------------------------------------|----------------------------|-----|--------|----------------------------------------|----|-----|-----|
| V                                                       | Cb | Ti  |                                      |                                      | Boiling HCl                |     |        | Boiling H <sub>2</sub> SO <sub>4</sub> |    |     |     |
|                                                         |    | 5%  | 10%                                  | 15%                                  | 5%                         | 10% | 20%    | 30%                                    |    |     |     |
| 70                                                      | 30 | —   | 2                                    | 737                                  | 18                         | 49  | 163    | 18                                     | 28 | 45  | 76  |
| 60                                                      | 40 | —   | <1                                   | 116                                  | 14                         | 39  | 104    | 14                                     | 25 | 35  | 64  |
| 50                                                      | 50 | —   | <1                                   | 17                                   | 8                          | 50  | 83     | 11                                     | 17 | 31  | 63  |
| 50                                                      | 40 | 10  | <1                                   | 18                                   | 11                         | 46  | 129    | 15                                     | 32 | 56  | 109 |
| 50                                                      | 30 | 20  | <1                                   | 18                                   | 17                         | 75  | 251    | 33                                     | 58 | 118 | 196 |
| 40                                                      | 40 | 20  | <1                                   | 9                                    | 13                         | 51  | 192    | 22                                     | 51 | 94  | 153 |
| 100                                                     | —  | —   | Diss                                 | 40                                   | 200+                       | —   | —      | 40                                     | —  | —   | 180 |
|                                                         |    | 100 | <1                                   | 4-21                                 | >1,000                     | —   | >1,000 | —                                      | —  | —   | —   |
| Prior art alloys (nominal compositions, percent by wt.) |    |     |                                      |                                      |                            |     |        |                                        |    |     |     |
| 99.4 Ti, 0.2 Pd                                         | —  | —   | 1                                    | 4-26                                 | 7                          | 32  | 267    | 20                                     | 69 | 207 | —   |
| 60 Ni, 30 Mo, 5 Fe, rem. Mn and Si                      | —  | —   | —                                    | —                                    | 7                          | 9   | 14     | 1                                      | 2  | 2   | 2   |
| 56 Ni, 16 Mo, 16 Cr, 5 W, 5 Fe, rem. Mn and Si          | —  | —   | 1                                    | —                                    | —                          | 332 | —      | 21                                     | 33 | —   | —   |
| 304 Stainless Steel                                     | —  | —   | —                                    | 10                                   | —                          | —   | —      | —                                      | —  | —   | —   |

oxygen at elevated temperatures is obtained as well as a corresponding increase in the resistance of said alloy to aqueous oxidizing media.

As an example illustrating the foregoing, reference is made to Table I which sets forth data on the corrosion behaviour in various aqueous media of the alloys of the present invention; and for comparison, pure vanadium, and select number of outstanding corrosion resistant alloys of the prior art are tabulated.

It may be seen from the foregoing table that alloys representative of this invention possess corrosion resistance comparable to, if not more superior than, the best corrosion resistant alloys available.

It has further been found that chromium, aluminum, cobalt, nickel, zirconium, hafnium or iron may be added to the alloy to augment the strength as well as enhance the oxidation resistance.

For examples illustrating the foregoing, reference may be had to the following Table II and Table III and Table IV. Table II sets forth data on the oxidation behaviour at elevated temperatures of the present alloys.

Table III

## OXIDATION RATES OF VANADIUM-COLUMBIUM ALLOYS

| 5  | Composition, percent by wt. |    |    |       | Rate of steady-state oxidation in pure oxygen (mg./cm. <sup>2</sup> /hr.) |         |         |
|----|-----------------------------|----|----|-------|---------------------------------------------------------------------------|---------|---------|
|    | V                           | Cb | Ti | Other | 700° C.                                                                   | 800° C. | 900° C. |
| 10 | 70                          | 30 |    |       | 14.4                                                                      | 32      |         |
|    | 60                          | 40 |    |       | 9.8                                                                       | 57.4    | 64.0    |
|    | 50                          | 50 |    |       | 8.7                                                                       | 312.0   | 510.0   |
|    | 50                          | 30 | 20 |       | 6.4                                                                       | 18.2    | 41.3    |
|    | 50                          | 40 | 10 |       | 7.2                                                                       | 9.0     | 18.8    |
|    | 40                          | 40 | 20 |       | 13.1                                                                      | 54.2    | 115.0   |
|    | 55                          | 40 |    | 5 Al. | 10.5                                                                      | 18.8    | 38.6    |
|    | 65                          | 40 |    | 5 Cr. | 20.5                                                                      | 15.0    | 24.0    |
|    | 55                          | 40 |    | 5 Si  | 20.9                                                                      | 58.8    |         |
|    | 50                          | 35 | 10 | 5 Al. | 8.6                                                                       | 9.6     | 20.0    |
| 15 | 55                          | 30 | 10 | 5 Si  | 18.0                                                                      | 13.1    | 14.9    |
|    | 48                          | 40 | 10 | 2 Si  | 7.1                                                                       | 14.1    | 48.7    |
|    | 45                          | 40 | 10 | 5 Si  | 7.7                                                                       | 12.2    | 18.7    |
|    |                             |    |    |       |                                                                           |         |         |

Table IV and II set forth data on tensile strength and creep-rupture strength at elevated temperatures of the present alloys. Pure vanadium and 310 type stainless steel are included for purposes of comparison.

Table IV

## 25 MECHANICAL PROPERTIES OF VANADIUM-COLUMBIUM ALLOYS

| 30                                         | Alloy composition weight percent |    |    |                                       | Ultimate tensile strength in p.s.i. at— |                       |                       |
|--------------------------------------------|----------------------------------|----|----|---------------------------------------|-----------------------------------------|-----------------------|-----------------------|
|                                            | V                                | Cb | Ti | Other                                 | 400° C.                                 | 700° C.               | 1000° C.              |
| 35                                         | 70                               | 30 |    |                                       | 127,000                                 |                       |                       |
|                                            | 60                               | 40 |    |                                       | 153,000                                 | 103,200               | 34,800                |
|                                            | 50                               | 40 | 10 |                                       | 98,500                                  | 91,800                |                       |
|                                            | 49                               | 40 | 10 | 1 Si                                  | 99,800                                  | 121,000               | 12,800                |
|                                            | 45                               | 40 | 10 | 5 Al                                  | 91,200                                  |                       | 7,960                 |
|                                            |                                  |    |    |                                       |                                         |                       |                       |
|                                            | Prior art alloys                 |    |    |                                       |                                         |                       |                       |
|                                            | Pure vanadium                    |    |    |                                       | 52,500                                  | 20,000                | 7,500                 |
|                                            | 310 Stainless Steel              |    |    |                                       | 80,000                                  | 50,000                | 17,000                |
|                                            |                                  |    |    |                                       |                                         |                       |                       |
| Table V                                    |                                  |    |    |                                       |                                         |                       |                       |
| CREEP PROPERTIES OF V-Cb ALLOYS AT 700° C. |                                  |    |    |                                       |                                         |                       |                       |
| Alloy composition wt. percent              |                                  |    |    | Minimum creep rate (in./in./hr.) for— |                                         |                       |                       |
|                                            |                                  |    |    | 75,000 p.s.i.                         | 90,000 p.s.i.                           | 100,000 p.s.i.        |                       |
| 60 V-40 Cb                                 |                                  |    |    |                                       |                                         |                       | $1.05 \times 10^{-4}$ |
| 50 V-40 Cb-10 Ti                           |                                  |    |    | $3.58 \times 10^{-4}$                 | $1.15 \times 10^{-4}$                   | $1.0 \times 10^{-4}$  |                       |
| 49 V-40 Cb-10 Ti-1 Si                      |                                  |    |    | $8.0 \times 10^{-5}$                  | $1.7 \times 10^{-4}$                    | $1.85 \times 10^{-4}$ |                       |

Table VI shows the effect of processing variables on the mechanical properties of the alloys of the present invention. All the alloys in the swaged condition have previously been extruded at 4:1 reduction at 1100 to 1200° C. All tensile tests were conducted at 0.02<sup>-1</sup> sec. strain rates. In the following table C.W. is used to designate cold worked.

Table VI

EFFECT OF PROCESSING VARIABLES ON MECHANICAL PROPERTIES<sup>1</sup>

| Alloy composition, wt. percent |    |    | Swaged condition | Annealed   |           | R.T., 0.2%                      |                               |            | 700° C., 0.2%                   |                               |            | 1000° C., 0.2%                  |                               |            | 1200° C., 0.2%                  |                               |            |
|--------------------------------|----|----|------------------|------------|-----------|---------------------------------|-------------------------------|------------|---------------------------------|-------------------------------|------------|---------------------------------|-------------------------------|------------|---------------------------------|-------------------------------|------------|
| V                              | Cb | Ti |                  | Temp., °C. | Time, hr. | U.T.S., p.s.i. $\times 10^{-3}$ | Y.S., p.s.i. $\times 10^{-3}$ | E, percent | U.T.S., p.s.i. $\times 10^{-3}$ | Y.S., p.s.i. $\times 10^{-3}$ | E, percent | U.T.S., p.s.i. $\times 10^{-3}$ | Y.S., p.s.i. $\times 10^{-3}$ | E, percent | U.T.S., p.s.i. $\times 10^{-3}$ | Y.S., p.s.i. $\times 10^{-3}$ | E, percent |
| 70                             | 30 | 30 | 30% C.W.         |            |           |                                 |                               |            | 128.6                           | 109.6                         | 5.2        |                                 |                               |            |                                 |                               |            |
| 70                             | 30 | 50 | 50% 1100°C       | 1100       | 0.5       | 124.1                           | 125.6                         | 2.2        | 130.2                           | 112.0                         | 6.0        | 70.1                            | 63.7                          | 89         | 23.2                            | 22.4                          | 43.6       |
| 70                             | 30 | 50 | 50% 1100°C       | 1200       | 0.5       | 123.8                           | 118.2                         | 2.0        | 121.7                           | 90.7                          | 69.0       | 68.2                            | 65.0                          | 72         |                                 |                               |            |
| 70                             | 30 | 50 | 50% 1100°C       | 1300       | 0.5       | 123.6                           | 114.7                         | 5.0        | 126.0                           | 90.7                          | 25.0       |                                 |                               |            |                                 |                               |            |
| 60                             | 40 | 40 | 50% 1000°C       | 1000       | 0.5       | 143.3                           | 136.9                         | 2.0        |                                 |                               |            |                                 |                               |            |                                 |                               |            |
| 60                             | 40 | 40 | 50% 1000°C       | 1100       | 0.5       | 154.6                           | 141.6                         | 62.5       | 140.2                           | 131.8                         | 40.5       | 68.3                            | 63.0                          | 35.3       | 22.8                            | 22.3                          | 14.0       |
| 60                             | 40 | 40 | 50% 1000°C       | 1300       | 0.5       | 125.8                           | 115.3                         | 7.7        | 86.7                            | 75.5                          | 2.8        |                                 |                               |            | 19.8                            | 19.0                          | 21.1       |
| 50                             | 40 | 10 | 40% C.W.         |            |           | 181.0                           | 177.2                         | 4.0        |                                 |                               |            |                                 |                               |            |                                 |                               |            |

<sup>1</sup> All tests performed at 0.02<sup>-1</sup> sec. strain rate.

As may be observed from the foregoing Table II the present alloys exhibit remarkable superiority in oxidation resistance at elevated temperatures over pure vanadium. It is further noted that the columbium-titanium-vanadium alloy shows an outstanding increase in oxidation resistance. The resistance of the 45 weight percent vanadium, 40 weight percent columbium, 10 weight percent titanium and 5 weight percent silicon alloy is also notable.

It may be noted from Table IV that the binary and its modifications surpass both pure vanadium and type 310 stainless steel in tensile strength at elevated temperatures. Particularly noteworthy is the exceptional strength of the alloys containing 10 weight percent titanium and 1 weight percent silicon at 700° C.

The addition of silicon, beryllium, barium, and the lanthanides, increases the resistance of the resulting alloy to oxidation at elevated temperatures. Examples illustrating this may be had by reference to the aforementioned Table II. It may be further observed that additions of these elements appreciably augment the mechanical strength. This fact is amply demonstrated in both Table IV and Table V. Table VII sets forth data on the stress rupture properties of the subject alloys. Two commercial alloys of outstanding high temperature strength and type 310 stainless steel are included for purposes of comparison.

Table VII

STRESS-RUPTURE PROPERTIES OF VANADIUM-COLUMBIUM ALLOYS UNDER HELIUM ATMOSPHERE

| Alloy composition, weight percent                      |    |    |       | Stress for 100-hour life at 700°C. |         |                |
|--------------------------------------------------------|----|----|-------|------------------------------------|---------|----------------|
| V                                                      | Cb | Ti | Other | Density, gm. lb./in. <sup>3</sup>  | p.s.i.  | p.s.i. density |
| 60                                                     | 40 |    |       | 0.25                               | 110,000 | 440,000        |
| 50                                                     | 40 | 10 |       | 0.24                               | 85,000  | 355,000        |
| 49                                                     | 40 | 10 | 1 Si  | 0.23                               | 90,000  | 390,000        |
| Prior art alloys nominal composition by weight percent |    |    |       |                                    |         |                |
| 20 Cr, 12 Co, 10 Mo, 3 Ti, 1.5 Al, Rem. Ni             |    |    |       | 0.290                              | 84,000  | 290,000        |
| 20 Cr, 20 Co, 5 Mo, 4 Fe, 3 Ti, 3 Al, Rem. Ni          |    |    |       | 0.290                              | 85,000  | 293,000        |
| 310 Stainless Steel                                    |    |    |       | 0.28                               | 20,000  | 71,500         |

The evidence of Table VII serves to demonstrate the outstanding strength and particularly the strength-to-weight ratio of the alloys of this invention. On this basis it is possible to conclude that said alloys have stress-rupture properties, on a density basis, well in excess of those of any other known material at 700° C.

In all the foregoing tables, the alloys of the present invention noted therein contain less than about 1 weight percent in the aggregate of carbon, oxygen and nitrogen. The alloys of the present invention can be prepared by any consumable or nonconsumable arc melting techniques

or any powder metallurgical process. The alloys can, of course, be processed also by forging, rolling, and standard extrusion. Although a primary reduction at elevated temperature is recommended, subsequent fabrication can be performed at temperatures as low as room temperature.

One of the most important novel aspects of these alloys is that they can be hot worked without the necessity of protective cover either from special coating or blanket of inert gas. This feature greatly simplifies and lessens the cost of fabrication.

From the foregoing it will be evident that alloys of the present invention exhibit excellent mechanical strength at elevated temperatures and in addition exhibit outstanding corrosion resistance to both aqueous and gaseous environments.

These alloys are particularly useful where extreme temperatures and operating conditions are met such as, for instance, those conditions which are associated with propulsion systems and nuclear reactors.

I claim:

1. An alloy comprising 25 to 40 weight percent columbium 3 to 15 weight percent titanium, 15 to 25 weight percent of at least one element selected from the group consisting of molybdenum, tantalum, tungsten and iron; up to 5 weight percent of at least one element selected from the group consisting of chromium, aluminum, cobalt, nickel, zirconium and hafnium; up to 3 weight percent of at least one element selected from the group consisting of silicon, beryllium, and the lanthanides; not more than 1 weight percent in the aggregate of carbon, oxygen and nitrogen; and the remainder vanadium in at least 40 weight percent, wherein the sum of said vanadium and said columbium comprises at least 65 weight percent in the aggregate.
2. An alloy consisting essentially of 25 to 40 weight percent columbium, 3 to 15 weight percent titanium; up to 5 weight percent of at least one element selected from the group consisting of chromium and aluminum; up to 3 weight percent silicon, less than about 1 weight percent in the aggregate of carbon, oxygen and nitrogen, and the remainder vanadium in at least 40 weight percent.
3. An alloy consisting of from 3 to 15% titanium, 25-40% columbium, balance vanadium.
4. An alloy comprising 40 weight percent columbium; 5 weight percent chromium; about 55 weight percent vanadium and less than about 1 weight percent in the aggregate of carbon, nitrogen and oxygen.

References Cited in the file of this patent  
UNITED STATES PATENTS

- 2,805,153 Rostoker ----- Sept. 3, 1957  
2,860,970 Thielemann ----- Nov. 18, 1958

## OTHER REFERENCES

- Transactions, American Society for Metals, vol. 46, pages 1156-1157, published in 1954 by the Society, Cleveland, Ohio.